

[54] ELECTRODE COMPRISING A POROUS SINTERED BODY

[75] Inventors: Ulrich Kümmel, Munich; Manfred Mair, Augsburg, both of Germany

[73] Assignee: Patent-Treuhand-Gesellschaft für elektrische Glühlampen mbH, Munich, Germany

[22] Filed: Sept. 12, 1973

[21] Appl. No.: 396,446

[30] Foreign Application Priority Data

Sept. 18, 1972 Germany..... 2245717

[52] U.S. Cl..... 313/346 R; 29/25.14; 29/25.17; 313/311; 313/218

[51] Int. Cl.<sup>2</sup>..... H01J 1/14; H01J 19/06

[58] Field of Search ..... 313/311, 346, 357, 218; 29/25.14, 25.17

[56] References Cited

UNITED STATES PATENTS

- |           |         |                   |             |
|-----------|---------|-------------------|-------------|
| 2,492,142 | 12/1949 | Germeshausen..... | 313/346 R   |
| 2,830,218 | 4/1958  | Beggs.....        | 313/346 R   |
| 2,975,322 | 3/1961  | Cockrill.....     | 313/346 R   |
| 3,010,046 | 11/1961 | Dailey et al..... | 313/346 R   |
| 3,076,915 | 2/1963  | Gal et al.....    | 313/346 R   |
| 3,244,929 | 4/1966  | Kuhl.....         | 313/346 R X |

|           |        |               |           |
|-----------|--------|---------------|-----------|
| 3,558,966 | 1/1971 | Hill .....    | 313/346 R |
| 3,656,020 | 4/1972 | Cronin .....  | 313/311   |
| 3,661,536 | 5/1972 | Shimizu ..... | 313/311   |

Primary Examiner—Saxfield Chatmon, Jr.

Attorney, Agent, or Firm—Flynn & Frishauf

[57]

ABSTRACT

A sintered electrode adapted to operate with an electric discharge arc appended to an outer surface thereof as one of the electrode components of high temperature discharge lamps such as gaseous and vapor discharge lamps and more particularly high-pressure discharge lamps. The electrode comprises a central electrode rod having one portion substantially enclosed by two contiguous porous sintered zones each of which has an exposed outer surface. The exposed outer surface of the first of the two zones is positioned in the direction of the arc discharge during operation of the lamp and is closer proximity thereto during operation than the outer surface of the second zone. The first zone consists of a refractory material which has been sintered at a temperature higher than the temperature of the arc discharge to form a sintered interconnected porous material. The second zone consists of a sintered porous mixture of refractory material and emissive material.

2

21 Claims, 2 Drawing Figures





## ELECTRODE COMPRISING A POROUS SINTERED BODY

Electrodes having a sintered body are known. British Pat. No. 943,535 discloses a porous cathode body composed of tungsten which is saturated with an emissive substance. The cathode body also contains a second emissive substance having a lower electron work function disposed in recesses of the surface facing the arc discharge. This second emissive substance is used for initiation of the arc discharge. U.S. Pat. No. 3,244,929 discloses a sintered electrode body composed of several zones formed from different emissive mixtures. These mixtures are compressed and sintered about an electrode rod. The zones of higher electron work function and heat resistance are provided in the direction of the space which contains the discharge arc during operation. The zones having a lower electron work function are positioned away from the space adapted to be occupied by the arc discharge during operation, i.e., the zones of lower work function are at the other side of the electrode.

The emissive characteristic of an electrode which are most satisfactory during operation of the arc discharge are different from the emissive characteristics which are most satisfactory for initiating said arc discharge. The aforescribed prior art constructions provide electrodes having at least two surfaces having different emissive characteristics, one more suitable for initiation of the arc, and the other more suitable for operation of the arc. The present invention provides an improved electrode for discharge lamps having superior characteristics for initiation of the arc and operation of the arc.

### SUBJECT MATTER OF THE INVENTION

The present invention provides a sintered electrode for use in gaseous and/or vapor discharge lamps and, particularly, high-pressure lamps. The sintered electrode contains a central electrode rod having one portion substantially enclosed by two contiguous porous sintered zones each of which has an exposed outer surface. The exposed outer surface of the first zone is positioned in the direction of the electric arc discharge during operation of the lamp and in closer proximity thereto during operation than the outer surface of the second zone. The first zone consists of a sintered interconnected porous refractory material which has been sintered at a higher temperature than the temperature reached during service of the discharge lamp, i.e., at a higher temperature than the temperature of the arc discharge proximate the electrode surface. The second zone consists of a sintered mixture of refractory material and emissive material.

Both zones may be formed by sintering high temperature refractory metals, e.g., tungsten, or high temperature refractory metallic compounds, e.g., zirconium carbide, lanthanum boride, etc.

The first zone which does not contain emissive material during preparation of the electrode has a density of between 8 and 16 grams per cubic centimeter when using tungsten as the refractory material. The preferred density is from 10 to 14 grams per cubic centimeter. The second sintered zone contains an emissive substance with the refractory material. The relative amounts, for example of a refractory material such as tungsten, and the emissive material vary from about 30

to 70 percent by weight of refractory material to about 70 to 30 percent by weight of the emissive material. The percent by weight is based on the total. The preferred ratio is 50—50 weight percent of each.

- 5 The emissive material or substance includes those known to the prior art to be suitable for this purpose, such as the oxides of barium, calcium and thorium, and also barium cerate.
- 10 The first zone has a sintered structure of interconnected pores. The second zone which is contiguous with the first zone has a refractory metal skeleton and contains emissive material in interconnected pores. Because of the contiguous relationship of the two zones, the emissive material from the second zone flows into the outer first zone and to the surface thereof during operation. This prevents sputtering of the refractory material at the position or positions at which the arc discharge appends during operation of the lamp. The terms "appends" and "appended" refer to the position at which the arc discharge makes contact with the surface of the electrode during operation of the lamp and also the position at which contact is made during ignition of the lamp. As noted, the arc appends to the second zone during initiation of the discharge and occurs immediately when the arc strikes or forms. The arc appends to the outer surface of the first zone during operation of the lamp. In a preferred embodiment of the present invention, the second zone is positioned within 15 a cavity of the first zone which is shaped as a cap over the second zone. The outer surface of the first zone, i.e., the cap, may have such shapes as a cylindrical surface, a conical surface or a frustoconical shape. The opening of the cap in which the second zone material is encompassed faces away from the direction of the arc discharge during operation of the lamp.
- 20
- 25
- 30
- 35

- The electrode rod which is preferably centrally positioned in the sintered electrode either protrudes with its end extending through the cap-shaped first zone in 40 the direction of the arc discharge during operation, or it may terminate with the cap-shaped zone. This preferred embodiment provides a second zone for initiation of the arc having an exposed surface of large area 45 extending in the direction away from the arc discharge during operation.

The invention will be described by way of example with reference to the accompanying drawings wherein:

FIG. 1 is a section through one preferred embodiment of the electrode; and

FIG. 2 is a section through another preferred embodiment of the electrode.

- In FIG. 1 the electrode rod 1 of thoriated tungsten having a diameter of 1.2 mm projects with its tip 2 approximately 1.5 mm out of the sintered body 3. The sintered body 3 is of cylindrical shape. Its length of about 5 mm is slightly larger than its diameter. It comprises a first zone 4 and a second zone 5. The first zone 4 has the shape of a cylindrical cap with bell-shaped cavity 6. It is made of finely sintered porous tungsten with a density of 12 g/cc. The cavity is almost completely filled with a sintered emissive mixture of 50 wt. percent of tungsten and 50 wt. percent of a mixture of oxides of barium, calcium, and thorium which forms the second zone 5. The outer surface 7 of the first zone 4 within the lamp is located more closely to the discharge than the outer surface 8 of the second zone 5.
- 55
- 60
- 65

In FIG. 2 the first zone 4 has the shape of a conical cap 9. The electrode rod 1 terminates with its tip 2 within the surface boundary of cap 9.

The sintered electrodes of the present invention are advantageous prepared using powder metallurgic techniques. The first electrode zone has particularly superior mechanical and high temperature properties. The sintered material having interconnected pores is suitably prepared by admixing the refractory material, e.g., tungsten, or zirconium carbide, with a powdered material which will not alloy with the refractory material and which has a sufficiently low boiling point so that it will vaporize during sintering. Suitable low temperature materials include zinc, copper, gold, etc. When using tungsten as the refractory material, zinc is particularly suited as the low boiling point material because it additionally functions as a pressing aid during the pressing of the shaped body.

The mixture of the refractory material and the low boiling point material is pressed to the desired shape using conventional powder metallurgical techniques. The electrode rod may be pressed into the sintered body at the same time. The slug is sintered at a temperature above the vaporization temperature of the low boiling point material. During this first sintering step, the low boiling material evaporates leaving a sintered, porous, skeletal structure which is then subjected to a higher temperature sintering, with temperatures up to 2600°C. The high degree of porosity and the interconnected porous structure is maintained during such high temperature sintering. Scan electron microscopic photographs of electrodes so prepared disclose that the bridges between the individual grains forming the slug, attain a width during high temperature sintering almost sufficient to match the grain dimensions. This accounts for the high temperature strength. Such structure is attained while maintaining the interconnected pore structure.

The second zone is prepared utilizing a powder mixture of the refractory material, e.g., a metal such as tungsten, and the emissive material. This powder mixture may be attached to the first zone. When the first zone is in the form of a hollow-shaped body, the powder mixture of the second zone material may be introduced into the cavity of the first zone and the two sintered together at a lower temperature of up to about 2000°C. This forms the emitter-containing second zone. During the preparation of the first zone, the sintering may be in two sequential steps as aforescribed, or in a single sintering wherein the evaporation of the low boiling point material and the final sintering are achieved in a single continuous sintering operation.

When utilizing certain refractory materials, such as tungsten, an inert atmosphere or vacuum is required to prevent oxidation, as is well known in the art.

The advantage of sintered electrodes when compared with wire coil electrodes is that the sintered electrodes are cheaper and more simple to manufacture. However, their stability at high electrical and thermal loads has been insufficient to attain a warranted lifetime of more than 5000 hours. Accordingly, they were not used in lamps with a wattage input exceeding 125 watts.

The electrodes of the present invention have superior service characteristics and are suitable for use in discharge lamps with a wattage input of 400 watts and even higher. This is possible because the high sintering

temperature not only improves the mechanical properties and high temperature stability of the porous structure, but also improves the electrical conductivity thereof. As noted, the high temperature at which the first zone of the electrode is sintered results in a structure having high temperature stability without sintering resulting in closing of the pores even with a high load. As a consequence, the supply of successive doses of emissive material to the surface of the first zone from the second zone is assured during operation.

Due to the bell shape of the preferred embodiment of the present invention and the consequent large area provided at which the arc discharge may append during start-up of the lamp, and the positioning of this large area at the rear of the electrode away from the arc discharge area during operation, there results a favorable rapid heating of the space behind the electrode as a consequence of the high current intensity during start-up and provides a rapid transition of the arc discharge to the lower current density station high-pressure phase. The low heat capacity of the electrode produced in accordance with the present invention contributes to this effect. The bell-shaped cavity of the preferred embodiments results in effective protection of the emitter-rich second zone during stationary operation of the lamp.

When using an electrode with tungsten as the refractory material in a lamp in which the temperature immediately at the position where the arc discharge touches the electrode is, for example, about 2000°C, the sintering temperature of the first zone preferably ranges between 2400° and 2600°C. The sintering temperature of the second zone which includes emissive material of preferably barium oxide 19.5 percent by wt., calcium oxide 5.5 and thorium oxide 75.0 is between 1600° and 2000°C.

We claim:

1. A sintered electrode for discharge lamps adapted to operate with an electric discharge arc appended to an outer surface thereof, comprising a central electrode rod having one portion substantially enclosed by first and second contiguous porous sintered zones each of which has an exposed surface, said exposed surface of the said first zone being positioned in the direction of the arc discharge during operation of the lamp and in closer proximity thereto during operation than said exposed surface of said second zone, said first zone consisting of interconnected porous material refractory sintered at a temperature between 2400°C and 2600°C, and said second zone consisting of a sintered porous mixture of refractory material and emissive material.

2. The sintered electrode of claim 1 wherein said refractory material of said first and said second zones is a high temperature refractory metal.

3. The sintered electrode of claim 2 wherein said high temperature refractory metal is tungsten.

4. The sintered electrode of claim 3 wherein said first zone has a density of from 8 to 16 g/cc.

5. The sintered electrode of claim 4 wherein said second zone consists of tungsten and an emissive material in relative amounts of from 30-70 percent by weight of tungsten to 70-30 percent of said emissive material.

6. The sintered electrode of claim 5 wherein said first zone has a density of from 10-14 g/cc.

7. The sintered electrode of claim 6 wherein said second zone contains tungsten and emissive material in an amount of about 50 percent of each.

8. The sintered electrode of claim 7 wherein said emissive material is at least one compound selected from the group consisting of barium oxide, calcium oxide, thorium oxide, and barium cerate.

9. The sintered electrode of claim 8 wherein said first zone is formed in the shape of a bell-shaped cap with said electrode rod protruding from the open end of said cap and with said second zone positioned within the cavity of said cap.

10. The sintered electrode of claim 9 wherein said electrode rod also protrudes through the other end of said cap-shaped first zone.

11. The sintered electrode of claim 1 wherein said high temperature refractory metal is tungsten.

12. The sintered electrode of claim 1 wherein said emissive material is at least one compound selected from the group consisting of barium oxide, calcium oxide, thorium oxide, and barium cerate.

13. The sintered electrode of claim 1 wherein said second zone consists of tungsten and an emissive material in relative amounts of from 30-70 percent by weight of tungsten to 70-30 percent of said emissive material.

14. The sintered electrode of claim 1 wherein said first zone is formed in the shape of a bell-shaped cap with said electrode rod protruding from the open end of said cap and with said second zone positioned within the cavity of said cap.

15. The sintered electrode of claim 1 wherein said electrode rod also protrudes through the other end of said cap-shaped first zone.

16. A method of manufacturing a sintered electrode for discharge lamps adapted to operate with an electric discharge arc appended to an outer surface thereof having a central electrode rod with one portion substantially enclosed by first and second contiguous porous sintered zones each of which has an exposed surface, said exposed surface of the said first zone being positioned in the direction of the arc discharge during operation of the lamp and in closer proximity thereto during operation than said exposed surface of said second zone; comprising admixing a powdered refractory

material with a low boiling point material which does not alloy with said refractory material and which vaporizes at the sintering temperature of said refractory material; compressing said admixture in a shaped die around said electrode rod to form a pressed compact surrounding said electrode rod; sintering said pressed compact and electrode rod at a temperature above the vaporization temperature of said low boiling point material whereby said low boiling point material completely vaporizes; and then sintering at a higher temperature up to about 2600°C to obtain an interconnected porous first zone substantially enclosing a portion of said central electrode rod having high mechanical and high temperature properties during high temperature service; and forming a shaped admixture of refractory material and said emissive material in the cavity of said bell-shaped sintered refractory material and sintering at a lower temperature up to about 2000°C.

17. The method of claim 16 wherein said electrode rod is thoriated tungsten, said refractory material in said first zone is selected from the group consisting of tungsten, zirconium carbide and lanthanum boride, and said low boiling point material is zinc.

18. The process of claim 17 wherein said refractory material is tungsten and wherein said tungsten is sintered at a temperature between 2400°C and 2600°C to obtain said interconnected porous first zone.

19. The process of claim 18 wherein said emissive material consists of barium oxide, calcium oxide and thorium oxide, and wherein the final sintering is at a temperature between 1600°C and 2000°C.

20. The sintered electrode of claim 7 wherein said emissive material consists of 19.5 percent by weight of barium oxide, 5.5 percent of calcium oxide and 75 percent of thorium oxide.

21. The sintered electrode of claim 11 wherein said second zone comprises 50 percent tungsten and 50 percent emissive material and said emissive material consists of 19.5 percent by weight of barium oxide, 5.5 percent of calcium oxide and 75 percent of thorium oxide.

\* \* \* \* \*